

1,272,566.

D. M. SUTHERLAND, JR.  
MANUFACTURE OF PULP BOARDS.  
APPLICATION FILED DEC. 20, 1913.

Patented July 16, 1918.

2 SHEETS—SHEET 1.



1,272,566.

D. M. SUTHERLAND, JR.  
MANUFACTURE OF PULP BOARDS.  
APPLICATION FILED DEC. 20, 1913.

Patented July 16, 1918.

2 SHEETS—SHEET 2.



G. V. Rasmussen  
John A. Ferguson

DANIEL M. SUTHERLAND JR.  
BY  
Biesen & Knauth  
ATTORNEYS

# UNITED STATES PATENT OFFICE.

DANIEL MANSON SUTHERLAND, JR., OF TRENTON, NEW JERSEY, ASSIGNOR TO THE AGASOTE MILBOARD CO., OF EWING TOWNSHIP, NEW JERSEY, A CORPORATION OF NEW JERSEY.

## MANUFACTURE OF PULP BOARDS.

1,272,566.

Specification of Letters Patent. Patented July 16, 1918.

Application filed December 20, 1913. Serial No. 807,867.

*To all whom it may concern:*

Be it known that I, DANIEL MANSON SUTHERLAND, Jr., a subject of the King of Great Britain, and a resident of Trenton, 5 Mercer county, New Jersey, have invented certain new and useful Improvements in the Manufacture of Pulp Boards, of which the following, taken in connection with the accompanying drawings, is a specification.

10 My invention relates to the manufacture of compressed pulp articles such as pulp boards and has for its objects to produce superior articles of such kind by means of atmospheric pressure; to balance such pressure so as to eliminate heavy and expensive apparatus; to felt together the pulp fibers to a maximum degree by imparting to them a vibratory movement during the removal of the water from the pulp; and to provide 15 an apparatus for such manufacture which is light, inexpensive and easy of construction and operation and which is capable of producing the finished article in a minimum of time. Other objects will be specifically 20 pointed out or will otherwise appear in the following description of my invention, an embodiment of the apparatus of which is shown in the accompanying drawings in which.

25 Figure 1 is a side elevation of a pulp board forming apparatus.

30 Fig. 2 is a front elevation thereof.

Fig. 3 is a cross section of a portion of the lower mold and

35 Fig. 4 is a fragmentary plan view of said mold.

The molds of the apparatus illustrated are mounted on a framework consisting of four vertical posts 5 supported on a suitable 40 foundation and connected together at their tops by the horizontal beams 6. Firmly secured to the posts 5 near the lower extremities thereof are the two channel irons 7, one of which extends horizontally between 45 the two front posts 5 and the other of which extends in like manner and at the same level between the two back posts 5. The upper surfaces of these channels form supporting tracks for the wheels 8 of the lower mold frame 9 upon which the lower mold 10 is supported. At one side of the framework for example on extensions of the tracks 7 a shaft 11 is suitably mounted; this shaft 50 may be rotated by the gear 12 which may be driven in any desired way as, for instance,

by means of an electric motor, and said shaft is provided at one or more points with cams 13 each of which coöperates with an eccentric 14, one end of which is pivoted to the lug 14' on the lower mold frame 9. It 60 will be readily understood that when the shaft 11 is rotated, the mold frame and the mold will be given a vibratory movement, the wheels 8 running to and fro upon the tracks 7. A system of piping 15 leading 65 from the bottom of the mold 10 at a plurality of distributed points, and having a flexible portion 15' so as to allow of the vibration of the mold, connects with a suitable 70 vacuum pump or other vacuum producing means located externally of the board forming apparatus.

The bottom of the mold 10 is composed of longitudinal sections 10' (see Fig. 3) each having depending ribs along its sides by 75 the aid of which the sections are tightly secured together by the bolts 10''.

The upper surfaces of the sections 10' are provided with channels between the cross-shaped projections 16, the upper ends of 80 which are in the same horizontal plane. Above these projections is laid a fabric 16', preferably of metal, having a relatively coarse mesh and above this fabric is positioned another fabric 16'' the mesh of which 85 is relatively fine. Where the pipes of the suction system 15 are joined to the mold bottom, and above the ends of the pipes, a cap 17 is provided to prevent the sagging of the superposed fabrics. 90

The deckle of the mold 10 is formed at the sides of the mold into flow boxes 18 which extend preferably the whole length of the mold. At the inner side of each flow box an overflow wall 18' is provided, the 95 upper edge of said wall being level. Within the box a downwardly extending baffle plate 18'' is provided, the lower end of said plate being below the upper edge of said overflow wall. 100

Upon the beams 6 a pulp supply tank 19 is supported; the suspension of pulp in water which this tank is adapted to hold is stirred by a suitably operated stirrer 19'. From this tank a pulp conduit system 20 105 provided with a valve 21, leads to the pulp inlet pipe 22, extending along the side of each flow box. Short branches 22' extend from the pipes 22 into the flow boxes so as to discharge equal amounts of the pulp 110

liquid into the flow boxes behind the baffles. A flexible connection such as the rubber conduit 20' is provided in the system 20 so that this system will not prevent or hinder the vibration of the pulp receiving mold.

Vertically slidable on the posts 5 is the frame 23 which supports below it the upper mold 24. This mold may be in the form of a plate having a flat perforated lower surface in which are channels similar to those of the lower mold 10. A vacuum system 25 leads from a plurality of points of the mold 24 to a suction producing apparatus which may, if desired, be the same apparatus as that which produces suction in the system 15 for the lower mold. A flexible joint 25' may be inserted in the system 25.

The upper mold may be moved up and down by means of any suitable mechanism. As shown, this consists of vertical screws 26 which are guided in bearings 26' secured to the beams 7 and 6, the bearings being such as to prevent the longitudinal movement of the screws while allowing rotation thereof.

The frame 23 is suitably supported upon shafts 27 which are provided at their ends with wheels 28, adapted to run on the tracks 29 which may take the form of channel irons slidably supported by the posts 5. The tracks 29 rest upon flanged nuts 30 which are slidably but non-rotatably secured within suitable bearings 31, as by a pin and slot connection so that when the screws 26 are rotated, the tracks 29 and consequently the upper mold 24 and its frame 23 are raised or lowered. In alignment with the tracks 29 when they are raised to their uppermost position, as shown, are tracks 32, the ends 40 of which, adjacent to the tracks 29, are supported by the brackets 33 secured to posts 5.

The screws 26 are rotated uniformly by any suitable means, as, for instance, by the motor 34 suitably geared to the drive shaft 35 and through intermediate gearing to the several screws. The intermediate gearing may consist of bevel gears 36 and 36' on the shaft 35 and meshing respectively with bevel gears 37 and 37' mounted on the forward shaft 38 and the rearward shaft 38' respectively. On the ends of the shaft 38, bevel gears 39 and 40 are mounted each of which meshes with one of the bevel gears 41 on the ends of the forward screws 26. On the ends of the shaft 38' bevel gears 39' and 40' are mounted, each of which meshes with one of the bevel gears 41 on the ends of the rearward screws 26.

In the operation of the apparatus described above, pulp liquid is caused to flow into the flow boxes 18 by opening the valve 21, the upper mold being in a position remote from the lower mold. The flow boxes will fill uniformly until the liquid therein reaches the level of the upper edge of the

overflow walls 18' after which the pulp liquor will overflow and enter the mold evenly from both sides thereof, the advance line of the flow from each side moving toward the center line of the mold until the two flows meet at such line. The baffle 18' in each of the flow boxes prevents any disturbance which might make the flow uneven over the wall 18'. During the introduction of the pulp into the mold, a suction is produced in the system 15 so that, as will readily be understood, the water of the pulp is removed while at the same time the pulp is being deposited upon the perforated upper surface of the mold. The water clearance spaces in the mold formed between the X-shaped projections 16 form irregular paths for the drainage of the water and make such drainage slow until a vacuum is formed in the pipe system 15. For this reason the drainage and the deposit of pulp is very slight until the pulp liquid from the two boxes meet in the center of the mold. As soon as the liquid covers the entire surface of the mold, however, the drainage is comparatively very rapid. During the introduction of the pulp also, the mold is vibrated by means of the eccentrics 14. In this way the pulp particles floating in the liquor are vibrated back and forth, with the result that they are deposited in a more closely felted mass than if they were deposited quietly and due merely to the removal of the water.

When the proper amount of pulp has been supplied to produce a sheet of the desired content of pulp, the vibration of the lower mold is stopped and the upper mold 24 is lowered by operating the screws 26 until its lower surface comes into contact with the partly formed pulp board in the lower mold, suction being applied meanwhile to the pipe system 25. As soon as the upper mold comes into contact with the pulp, a vacuum is produced in the pipes 25 and the upper mold is suddenly forced downwardly by atmospheric pressure; the screws 26 are rotated sufficiently to allow of this sudden motion but are not further rotated to force the mold downwardly by mechanical pressure. The construction of the nuts 30 and the bearings 31 is such as to allow of a slight rotation of the screws after the contact of the upper mold with the pulp, without forcing the mold mechanically against the pulp.

Under such conditions the pulp board is compressed under atmospheric pressure exerted on the molds and moreover the water of the pulp is withdrawn both from the top and the bottom. It will be seen that since the pressure used is that of the atmosphere and particularly since the pressure is exerted on the two coacting molds in opposite directions and is therefore balanced, the framework and mechanism generally of the appa-

ratus is without strain due to the pressure and may be of light and inexpensive construction as compared with the well-known hydraulic press apparatus which has heretofore been employed for the manufacture of pulp articles. Furthermore, the use of atmospheric pressure in the manner described results in a stronger, better felted article than the product formed by forcing the pulp particles together quickly and under high pressure.

When the board has been formed in the manner described, the vacuum in the lower vacuum system 15 is broken as by opening the vent valve 42 for a moment; the screws 26 are then rotated to move the upper mold to its uppermost position, the newly formed board being retained by this mold because of the vacuum in the upper vacuum system 25. The mold when so positioned may now be run upon the tracks 32 to a point external to the apparatus where its load may be deposited by opening the vent valve 43, thus breaking the vacuum in the system 25 and allowing the board to fall.

While the finished board is being disengaged from the upper mold the lower mold is being filled with pulp liquid; the upper mold is then returned in time to complete the production of the board.

My invention is of especial adaptation to the production of large pulp board such as those having an area for example of sixty square feet and a thickness of one inch and is capable of producing such large boards with a percentage of air dry fiber as high as 35%. A massive and almost prohibitively expensive apparatus of the usual hydraulic press type would be required to produce a board of such dimensions and having such content of air dry fiber.

I claim:

1. The improvement in the art of making compressed pulp articles, which consists in placing the water-containing pulp in a lower mold, creating a reduced air pressure in said mold and simultaneously agitating said mold, whereby the bulk of the water is removed and the pulp fibers are closely felted together, then placing an upper mold in contact with the upper surface of said pulp and creating a reduced air pressure in said mold, the vacua of both molds being maintained simultaneously, whereby the molds are drawn together to compress the pulp and the expressed water of the pulp is removed from both sides thereof, substantially as and for the purpose described.

2. An apparatus for making compressed pulp articles comprising a mold for receiving the water-containing pulp, said mold being provided with a suction chamber, means

for vibrating said mold, a second mold also provided with a suction chamber, means for bringing the molds into juxtaposition and means for producing suction in said chambers.

3. An apparatus for making compressed pulp articles comprising a mold for receiving the water-containing pulp, said mold being provided with water drainage passages and means for vibrating said mold to augment the felting together of the pulp particles during the drainage of the water.

4. An apparatus for making compressed pulp articles, comprising a mold provided with a porous bottom and drainage passages leading therefrom, a flow box extending along one side of the mold and having an overflow wall, the upper edge of which is horizontal, and means for supplying water-containing pulp to said flow box.

5. An apparatus for making compressed pulp articles, comprising a mold provided with a porous bottom and drainage passages leading therefrom, a flow box extending along each side of the mold, each box having an overflow wall, the upper edge of which is horizontal, and means for supplying equal quantities of water-containing pulp simultaneously to each flow box.

6. An apparatus for making compressed pulp articles, comprising a mold provided with a porous bottom and drainage passages leading therefrom, a flow box extending along one side of the mold and having an overflow wall, the upper edge of which is horizontal and a baffle plate within said box and extending downwardly below said horizontal edge and means for supplying water-containing pulp to said flow box at the side of said baffle plate which is remote from said overflow wall.

7. An apparatus for making compressed pulp articles, comprising a mold provided with a porous bottom and drainage passages leading therefrom, a flow box extending along each side of the mold, each flow box having an overflow wall, the upper edge of which is horizontal and a baffle plate within each of said boxes and extending downwardly below said horizontal edge, and means for supplying equal quantities of water-containing pulp simultaneously to each flow box at the side of said baffle plate therein which is remote from said overflow wall.

In testimony whereof I have hereunto set my hand in the presence of two subscribing witnesses.

DANIEL MANSON SUTHERLAND, JR.

Witnesses:

JOHN A. FERGUSON,  
G. V. RASMUSSEN.